

No. 790,308.

Patented May 23, 1905.

# UNITED STATES PATENT OFFICE.

JOSEPH NENATOWICH, OF PAGE, NEW YORK.

## LUBRICATING COMPOUND.

SPECIFICATION forming part of Letters Patent No. 790,308, dated May 23, 1905.

Application filed September 29, 1904. Serial No. 226,582.

*To all whom it may concern:*

Be it known that I, JOSEPH NENATOWICH, a citizen of the United States, residing at Page, in the county of Lewis and State of New York, have invented certain new and useful Improvements in Lubricating Compounds, of which the following is a specification.

This invention relates to steam-engine lubricant, and consists of a novel compound comprising the following ingredients in about the proportions stated—*i. e.*, five ounces tallow, one ounce cylinder-oil, one ounce salt, two ounces soda, one ounce water, eight drams alum, two drams oil of cocoanut, two drams camphor.

The tallow is melted, after which the other ingredients are added. Textile or other fibrous material, such as asbestos cloth or wool, is saturated with the compound while in a heat-

ed and fluid state and is used in any well-known manner for packing the parts of engines.

The cylinder-oil forming an ingredient of the compound is refined petroleum, such as generally used for lubricating purposes.

Having thus described the invention, what is claimed as new is—

A lubricating compound for steam-engines consisting of tallow, cylinder-oil, salt, soda, water, alum, oil of cocoanut and camphor in about the proportions, substantially as specified.

In testimony whereof I affix my signature in presence of two witnesses.

JOSEPH NENATOWICH. [L. S.]  
Witnesses:

GEO. B. LOOMIS,  
L. E. BABCOCK.